

E. DU PONT.  
PROCESS OF MAKING EXPLOSIVE BLACK POWDER.  
APPLICATION FILED DEC. 29, 1915.

1,308,342.

Patented July 1, 1919.



WITNESS:

Robert Kitchel

INVENTOR  
Ernest du Pont  
BY  
Frank D. Bussur  
ATTORNEY.

# UNITED STATES PATENT OFFICE.

ERNEST DU PONT, OF WILMINGTON, DELAWARE, ASSIGNOR TO BALL GRAIN EXPLOSIVES COMPANY, OF WILMINGTON, DELAWARE, A CORPORATION OF DELAWARE.

## PROCESS OF MAKING EXPLOSIVE BLACK POWDER.

1,308,342.

Specification of Letters Patent.

Patented July 1, 1919.

Application filed December 29, 1915. Serial No. 69,167.

To all whom it may concern:

Be it known that I, ERNEST DU PONT, a citizen of the United States, residing at Wilmington, county of New Castle, and State 5 of Delaware, have invented a new and useful Improvement in Processes of Making Explosive Black Powder, of which the following is a full, clear, and exact description, reference being had to the accompanying 10 drawings, which form a part of this specification.

It is well understood that the manufacture of black powder is more or less dangerous; explosions sometimes resulting during 15 grinding and mixing, technically known as incorporation, and sometimes during the operation of pressing and forming the cakes or grains. In the latter operation the principal source of danger is undoubtedly the 20 great pressure—varying from 1500 to 2000 pounds per square inch—required to produce the desired finished product. Further, this high pressure produces such wear and tear of the parts in contact with the powder 25 that they have to be replaced very frequently.

The object of my invention is to so modify the process as to render the incorporating operation absolutely safe and to dispense 30 with the necessity of employing high pressure in the molding of the powder, thereby rendering this operation also absolutely safe and incidentally avoiding the expense and delay involved in the frequent substitution 35 of parts of the press.

The practice of the process involving my invention does not require the use of any special apparatus, but to aid in understanding of the process, I will describe the same 40 in connection with the accompanying drawings, in which—

Figure 1 is a vertical sectional view of a grinding and mixing mill; Fig. 2 a similar view of a stirring tank; and Fig. 3 a similar 45 view of a mold.

The mill shown in Fig. 1 is fully set forth and described in the du Pont and du Pont application, Serial No. 807,374, filed December 18, 1913, and comprises a cylinder *a* rev- 50 oluble on two pairs of wheels *b*, one pair of which is on a driving shaft *c*, the cylinder containing two heavy rollers *d*, and having axial openings *e* in the ends communicating with the interior of a box *f* sur- 55 rounding the cylinder.

The solid ingredients of the explosive,

namely, niter (either nitrate of potash or nitrate of soda), sulfur and charcoal, are ground together in the mill, which need not, however, be of the construction shown 60 in the drawings. In place of water there is employed a liquid which has no solvent or chemical effect upon the ingredients. Such a liquid is gasoline. The proportions of the solid ingredients may vary somewhat, but 65 a typical composition is one containing 75 parts by weight of nitrate of potash, 15 parts by weight of charcoal and 10 parts by weight of sulfur. The amount of gasoline or equivalent liquid added should be sufficient to 70 cover the mass and render it fluid during the process of grinding. This amount will vary with the particular liquid used and it will also vary with conditions; but, as an example, it may be stated that with 100 parts 75 of the above mixture of solid ingredients and with the grinding operation conducted at a temperature of 20° C., 100 parts by weight of gasoline has been found to suffice. To the above mixture should be added water, 80 say from 2.7 to 3.0 parts by weight, which is the same amount of water added in the ordinary so called dry process. The mill should be operated until all the solid materials are thoroughly ground together. 85

The mixture is then removed to a tank *g* provided with a stirring device *h*, the latter operating to keep the solid materials in suspension in the gasoline. It will be understood that no particular construction of apparatus is necessary to carry out this step of 90 the process.

Any measured quantity of the material that may be drawn off necessarily contains a definite quantity of the powder materials, 95 and such measured quantity so drawn off is poured into a mold and molded into a cake. In Fig. 3 is shown a simple form of mold that will be found efficacious, although no particular form of mold is essential. 100 The same comprises a tube *i* of metal of about one half inch internal diameter and two plungers *j*, *j'*. The plungers should be about as good a fit as a machinist would naturally make where free movement of the plungers within the tube is desired. It will be found that the exertion of a very slight pressure, such, for example, as can be exerted with comparatively light hand pressure is sufficient to compress the powder to 105 the extent desirable and to squeeze out the gasoline or at least a large portion of it; the 110

minute space between the tube *i* and the plungers *j*, *j'*, incident to the free sliding fit between them, being sufficient to allow the gasoline to escape.

- 5 The cake or rod of powder is then removed and dried at a temperature sufficient to drive off the remaining gasoline and the water. The proper temperature depends upon the time which it is desirable to take for drying.
- 10 Thus, if the temperature is high, say 100° C., the drying process takes but a very short time, but if the temperature is low, say 50° C., the time required to expel the moisture from the inside of the cake is relatively long.
- 15 Upon close examination and thorough test, the powder is found to have physical and other properties quite equal to, and in some respects superior to, those possessed by powder manufactured in any of the known
- 20 ways and pressed in a heavy press under a pressure of from 1500 to 2000 pounds per square inch. The molds will last indefinitely, the required pressure being so slight as to produce no appreciable wear and tear.
- 25 It will be understood that while other liquids having no solvent or chemical action upon the explosive ingredients may be used in place of gasoline, other liquids, such as alcohol, which is miscible with water, would
- 30 be incapable of use, because they would prevent the water from performing its function.

While, properly speaking, the mold has no selective action in eliminating the larger part of the gasoline and not the water, the fact is that only the gasoline will be therein eliminated. By reason of the solvent action of the water it is held as a coating around the particles of the material which it in part dissolves. Therefore, when the mass is coming 40 pressed in a mold which allows liquid to escape, or even should it be poured on a filter, the inactive liquid alone escapes.

Having now fully described my invention, what I claim and desire to protect by Letters Patent is:

1. The process of manufacturing explosive black powder which consists in incorporating the solid ingredients thereof with a liquid having no solvent or chemical action upon the ingredients and with water and then molding the explosive.

2. The process of manufacturing explosive black powder which consists in incorporating the solid ingredients thereof with a liquid having no solvent or chemical action upon the ingredients and with water of a weight less than that of said liquid, and then molding the explosive.

3. The process of manufacturing explosive black powder which consists in grinding and

mixing the solid ingredients thereof in the presence of a liquid having no solvent or chemical action upon the ingredient and in the presence of water, then stirring the mixture, and then molding the explosive.

4. The process of manufacturing pellets of explosive powder which consists in grinding together the solid ingredients thereof in a liquid which has no solvent or chemical action upon such of the ingredients as are to be ground, there being present a small percentage of a liquid having a solvent action on one ingredient and which therefore tends to resist dissociation therefrom, molding the explosive in a mold which permits a portion of the inactive liquid to escape, and subjecting the molded cakes to drying action at a temperature sufficient to dry off both the inactive and the solvent liquid.

5. The process of manufacturing explosive black powder which consists in incorporating the solid ingredients thereof with a liquid having no solvent or chemical action upon the ingredients and with water, the water having a solvent action upon a part of the powder and thereby tending to resist dissociation therefrom, then pressing the explosive in a mold and thereby expelling from the explosive more or less of the first named liquid, and then drying the molded product.

6. The process of manufacturing explosive black powder which consists in incorporating the solid ingredients thereof with a liquid having no solvent or chemical action upon the ingredients and with water of a weight between 1½ and 3½ per cent. of the weight of said solid ingredients.

7. The process of manufacturing pellets of explosive powder which consists in grinding together the solid ingredients thereof together, with from 1½ to 3½% of their weight of water, in gasoline, molding the powder in a mold from which the excess of gasoline can escape, the water by reason of its solvent action remaining in association with the powder, and subjecting the molded pellet to a drying action at a temperature sufficient to remove the gasoline and the water.

8. The process of manufacturing pellets of explosive powder, which consists in maintaining the mass, which has been previously ground, in suspension by agitation in gasoline, and measuring out definite volumes of the gasoline so that definite weights of pellets may be pre-determined.

In testimony of which invention, I have hereunto set my hand, at Philadelphia, Penna., on this 27th day of December, 1915.

ERNEST DU PONT.